

## UNITED STATES PATENT OFFICE

1,985,243

## METHOD OF PRODUCING ORNAMENTAL FABRIC

Camille Dreyfus, New York, N. Y., and Herbert Platt, Cumberland, Md., assignors to Celanese Corporation of America, a corporation of Delaware

No Drawing. Application December 20, 1928,  
Serial No. 327,471

5 Claims. (Cl. 28—1)

This invention relates to the preparation of fabrics containing yarns of organic derivatives of cellulose having on at least a part of the surface thereof a pebble or cockle effect produced by 5 chemical action.

An object of our invention is to produce cockle or pebble effects on at least part of the surface by the treatment of fabrics containing yarns of organic derivatives of cellulose and yarns of other fibres with a reagent that causes shrinkage of one kind of yarn and not of the other. Other 10 objects of our invention will appear from the following detailed description.

In accordance with our invention, we produce 15 ornamental effects on fabrics by treating mixed fabrics, which are so constructed that either the warp or weft or both contains both yarns of organic derivatives of cellulose and yarns of other fibres, with a reagent that causes shrinkage of 20 the one kind of yarn and not the other. Because of the shrinkage of one kind of yarn and not the other, the yarn that does shrink causes the other 25 yarn to cockle, thus producing novel effects.

The yarn made of the organic derivatives of cellulose may be made of organic esters such as cellulose acetate, cellulose formate, cellulose propionate and cellulose butyrate. This yarn may be sized or unsized prior to treatment with the shrinkage agent. The yarns of other fibres that 30 may be used may be made of silk, cotton, reconstituted cellulose, wool, etc. and these yarns may be of low twist or of high twist such as is used for creping.

As stated, the construction of the fabric should 35 be such that the yarns of one kind alternate either in the weft or in the warp with yarns of other kind. This alternation may be regular, that is for instance, an alternation of two yarns of cellulose acetate and two yarns of cotton, or it may 40 be in a form to produce checks, stripes or even complicated designs such as are produced by jacquard looms. As stated the alternation of the two kinds of yarns may occur either in the weft alone or in the warp alone or both in the weft 45 and in the warp. Thus the fabric may have a warp consisting wholly of yarns of cellulose acetate or consisting wholly of yarns of cotton, while the weft may be constructed by the alternation of two picks of cotton yarn and two picks of cellulose 50 acetate yarn. On the other hand the weft may consist wholly of either cellulose acetate yarn or wholly of say cotton yarn, while the warp is made up of two ends of cellulose acetate yarn alternating with two ends of cotton yarn. The 55 use of a mixed fabric, which is constructed of a

warp consisting wholly of one kind of yarn and a weft consisting wholly of another kind of yarn, will not produce the desired result, since on the shrinking of the one kind of yarn, say the weft, no cockling of the other yarn say the warp, will be produced, the only effect being that a fabric of closer weave is produced.

An example of a suitable reagent that causes the shrinking of one kind of yarn and not of the other is a solution of nitric acid. A solution of 10 nitric acid causes yarn of organic derivatives of cellulose such as cellulose acetate to shrink, while it does not cause yarns of cotton, reconstituted cellulose, silk or wool to shrink. The nitric acid may be of suitable concentration say from 15 28° to 60° Tw. and may be employed at temperatures of 0° to 60° C. Treatment of the fabric for 1 to 5 minutes or more is usually sufficient to produce the result. If the solution is at higher 20 temperature, a lower concentration of the nitric acid and less time is required.

The reagent for causing the shrinking may be applied to the whole surface of the fabric or it may be applied locally in the form of paste or by brushing or by spraying onto stencils, so that 25 the cockle effect is obtained in only certain predetermined portions of the fabric, whereby many ornamental effects may be produced.

By our invention pebble or cockle effects may be obtained on fabrics that are woven with ordinary 30 yarn by ordinary looms by the simple application of a chemical reagent. The fabric after treatment may be dyed, printed or finished in any suitable manner. In order further to illustrate our invention but without being limited 35 thereto the following specific example is given.

## Example

A fabric constructed of a warp consisting wholly of cellulose acetate yarn and a weft comprising two picks of cotton yarn alternating with two picks of cellulose acetate yarn is treated in a bath containing an aqueous solution of nitric acid of 38° Tw. at ordinary temperatures. The fabric is allowed to remain in the bath for 45 one minute, after which it is withdrawn, rinsed in cold water, dried, then scoured with soap, rinsed and dried. A fabric having a cockle surface is thus formed, this effect being produced by the buckling of the cotton yarn because of 50 the shrinking of the cellulose acetate yarn. This fabric may be dyed in any suitable manner, either to obtain a solid color, or in a cross-dyeing bath wherein one color is imparted to the cotton yarn and another color to the cellulose acetate yarn, 55

thus enhancing the ornamental effect. If reconstituted cellulose yarn (rayon) is substituted for the cotton yarn in the above fabric, similar results are obtained.

5 The term "alternating" as used in the appended claims is intended to include arranging the yarns in any regular or irregular manner.

It is to be understood that the foregoing detailed description is given merely by way of illustration, and that many variations may be made therein without departing from the spirit of our invention.

Having described our invention, what we claim and desire to secure by Letters Patent is:

- 15 1. Process of producing a fabric having cockle or pebble effects comprising treating a fabric having at least its warp or its weft constructed of yarns of organic derivatives of cellulose alternating with highly twisted yarns of non-vegetable fibres with a solution of nitric acid that causes the shrinkage of the organic derivative of cellulose yarn and no appreciable shrinkage of the other yarn.
- 20 2. Process of producing a fabric having cockle or pebble effects comprising treating a fabric having at least its warp or its weft constructed of yarns of organic derivatives of cellulose alternating with highly twisted yarns of natural silk with a solution of nitric acid that causes shrinkage of

the organic derivative of cellulose yarn and no appreciable shrinkage of the other yarn.

3. Process of producing a fabric having cockle or pebble effects comprising treating a fabric having at least its warp or its weft constructed of yarns of organic derivatives of cellulose alternating with highly twisted yarns of non-vegetable fibres with a solution of nitric acid of 28° to 50° Tw. that causes the shrinkage of the organic derivative of cellulose yarn and no appreciable shrinkage of the other yarn. 5

4. Process of producing a fabric having cockle or pebble effects comprising treating a fabric having at least its warp or its weft constructed of yarns of cellulose acetate alternating with highly twisted yarns of non-vegetable fibres with a solution of nitric acid of 28° to 50° Tw. that causes the shrinkage of the cellulose acetate yarn and no appreciable shrinkage of the other yarn. 10

5. Process of producing a fabric having cockle or pebble effects comprising treating a fabric having at least its warp or its weft constructed of yarns of cellulose acetate alternating with highly twisted yarns of natural silk with a solution of nitric acid of 28° to 50° Tw. that causes the shrinkage of the cellulose acetate yarn and no appreciable shrinkage of the natural silk yarn. 20 25

CAMILLE DREYFUS.  
HERBERT PLATT.